

## UNITED STATES PATENT OFFICE

2,537,526

## NITROPARAFFIN FUEL

John A. Hannum, Detroit, Mich., assignor, by  
mesne assignments, to Borg-Warner Corpora-  
tion, Chicago, Ill., a corporation of Illinois

No Drawing. Application July 30, 1946,  
Serial No. 687,213

11 Claims. (Cl. 52—1)

1

This invention relates to a self-sufficient mono-fuel or propellant for a prime mover that comprises a mixture of a combustible fuel component and an oxidizing agent. In particular it relates to such a self-sufficient fuel in which the fuel component is made up of one or more partially nitrated aliphatics of the nature of nitro and polynitro aliphatic hydrocarbons and in which an oxidizing agent selected from the group of fully nitrated aliphatics; e.g., tetranitromethane, is employed to supply the fuel component with all or substantially all the additional oxygen required for combustion of the mixture.

Propellants containing both fuel and oxygen in a combined form, also called self-sufficient fuels, have heretofore been proposed by Paul Winand in United States Patent 914,624, issued March 9, 1909. That patent teaches the use of a nitro benzol as a fuel and in particular the use in an engine of a mixture of a nitro benzol and tetranitromethane. One difficulty with such a fuel mixture is that it is highly explosive. Furthermore the Winand disclosure contemplates employing such "nitrated carbon compounds as contain a large proportion of carbon with respect to the hydrogen present." The heat value derived from the combustion of carbon is substantially less than results from the combustion of hydrogen with the result that practice based on the Winand disclosure, even if otherwise operable and advantageous, is subject to a lack of efficiency.

As distinguished from the prior art disclosure of using with tetranitromethane an aromatic hydrocarbon derivative, and particularly the nitrobenzols, the present invention contemplates the use therewith of nitro and polynitro aliphatic hydrocarbons and in particular mixtures that are non-brisant as hereafter defined. The fuel components are sufficiently safe to be handled by ordinary methods and are not substantially more dangerous to the user than gasoline and similar substances. They possess a high fuel value because, unlike aromatics, they generally have present more hydrogen than carbon. Furthermore they are relatively low in cost—less for instance than the nitrobenzols.

These fuel components contain a portion of the oxygen that is necessary for the combustion of the carbon and hydrogen atoms that form the basis of the fuel, the balance of the oxygen required for combustion being provided by a fully nitrated oxidizing agent that with the fuel component comprises the propellant or self-sufficient fuel.

2

While the self-sufficient fuel of the present invention is described as comprising a fuel component and an oxidizing agent, it is recognized that each may possess properties of the other. For example tetranitromethane, as an oxidant, gives off considerable heat when burned and nitromethane as a fuel contains a part of the oxygen required for its combustion. Such self-sufficient fuels are mono-fuels in the sense that, if desired, both oxidant and fuel can be supplied with safety to the point of combustion mixed as distinguished from those fuels where the ingredients are stored separately either because they are spontaneously combustible when mixed or for some other reason.

It is a general object of the present invention to provide a self-sufficient mono-fuel that is safe to handle, possesses a high fuel value and is of the proper viscosity and vapor pressure to provide a propellant of improved efficiency for the uses indicated herein. Another object is to provide a propellant comprising a fuel component selected from the group of nitro and polynitro aliphatic hydrocarbons and an oxidizing agent from the group of fully nitrated aliphatics to supply to the propellant the balance of oxygen required for combustion of the fuel. Still another object of the invention is to provide a fuel comprising an oxidizing agent and a non-brisant nitro or polynitro aliphatic hydrocarbon. A further object of the invention is to provide a self-sufficient fuel in which the fuel component may comprise a fortuitous mixture of mono-nitro aliphatics as derived from the reaction of propane and nitric acid in the vapor phase and an oxidizing agent. Still another object is to provide a mono-fuel in which both the oxidant and fuel component may be mixed in advance without spontaneous combustion or other harmful results. Other objects of the invention will become apparent as the description of the invention proceeds.

A propellant of the kind outlined above may be efficiently used for various purposes including a source of power for prime movers and more specifically such prime movers as gas turbines and reciprocating internal combustion engines. Gas turbines heretofore have been subject to a marked disadvantage in that it has been necessary to provide a compressor as an integral part of the unit in order that the requisite amount of oxygen might be made available for combustion of the fuel. The use of such a compressor decreases the over all operating efficiency and greatly increases the volume and weight of gas turbine in-

stallations. The fact that gas turbines in the past have derived their oxygen from the atmosphere imposed a marked ceiling limitation on aircraft driven by them because the atmosphere becomes more rarified as the altitude increases and has less available oxygen.

If a gas turbine could be provided with a suitable fuel which eliminated the foregoing disadvantages, its field of application would be considerably broadened. Fields in which it now has utility would be expanded and other fields in which its use is not now practical would be opened. At the present time gas turbines have found some use as stationary auxiliary equipment in power plants have been considered for use in driving railway locomotives. All of these uses would be expanded if the foregoing objections to the gas turbine as it now stands and to the fuel available for its use could be eliminated.

Although a prime use of the propellant described herein is for gas turbines it will be understood that it is susceptible to a wide variety of other uses. It may, for instance, be used in a reciprocating internal combustion engine and it may be used under a variety of circumstances as in aircraft, underwater craft, land vehicles and stationary installations. It can be used as a source of power for rockets. It is particularly useful at high altitudes where the rarified air offers little oxygen to support combustion. It can be used in many other situations where the burning of a self-sufficient fuel or propellant is desired to make available heat energy or gas pressure due to combustion.

As indicated above the fuel that is the subject matter of this invention comprises an oxidizing agent in the form of a fully nitrated aliphatic hydrocarbon and a fuel component in the form of a nitro or polynitro aliphatic hydrocarbon. The fuel component embodied in the propellant will be one such as nitromethane  $\text{CH}_3\text{NO}_2$ , that itself contains oxygen that may be used during combustion. It is contemplated that other fuel components from the class of nitro and polynitro aliphatic organic liquids may be used. Examples of such fuel components in addition to nitromethane are:

Nitroethane,  $\text{CH}_3\text{CH}_2\text{NO}_2$ .  
 1-nitropropane,  $\text{CH}_3\text{CH}_2\text{CH}_2\text{NO}_2$   
 2-nitropropane,  $(\text{CH}_3)_2\text{CH}\text{NO}_2$   
 1,1-dinitropropane,  $\text{C}_2\text{H}_5\text{CH}(\text{NO}_2)_2$   
 2,2-dinitropropane,  $(\text{CH}_3)_2\text{C}(\text{NO}_2)_2$   
 1,2-dinitropropane,  $\text{CH}_2\text{NO}_2\text{CHNO}_2\text{CH}_3$   
 1,3-dinitropropane,  $\text{CH}_2\text{NO}_2\text{CH}_2\text{CH}_2\text{NO}_2$   
 1,1-dinitroethane,  $\text{CH}_3\text{CH}(\text{NO}_2)_2$   
 1,2,3-trinitropropane,  $\text{CH}_2\text{NO}_2\text{CHNO}_2\text{CH}_2\text{NO}_2$   
 1,1,1-trinitropropane,  $\text{C}(\text{NO}_2)_3\text{CH}_2\text{CH}_3$

Such nitro and polynitro aliphatics included as fuels, as distinguished from oxidants, within the scope of this invention include mononitromethane, dinitroethane and trinitropropane and those nitroethanes and nitropropanes below them in oxygen content but no nitroethanes or nitropropanes that are higher in oxygen content, as for instance dinitromethane. These are all to be distinguished from aromatic fuels such as the nitrobenzols that are dangerous to handle even by skilled persons, to say nothing of persons who are not skilled in this art.

The fuel portion of the propellant mixture is limited to those nitro and polynitro aliphatics that contain not more than one nitro group; i. e., one molecule of oxygen, for each carbon atom present. Under many conditions for most effi-

cient use the fuel and oxidant will be combined in substantially stoichiometric proportions; i. e., the combining proportions required for combustion. This is the most economical use of the materials because after combustion there remains no appreciable amount of either unconsumed fuel or oxidant. An advantage of using nitromethane or a similar oxygen-containing fuel as listed above resides in the fact that it contains a considerable amount of oxygen that is available during combustion to burn part of the carbon or hydrogen in the fuel. This in turn does not require the inclusion in the propellant of as much oxidizing agent as would otherwise be necessary. These fuel components are non-brisant nitro and polynitro aliphatic compounds. When a fuel is said to be non-brisant within the terms of this disclosure it is meant that it may be burned in contact with chilled iron.

A propellant prepared in accord with the present invention preferably will contain a sufficient amount of oxidizing agent to provide with the oxygen of the fuel the required total amount of oxygen for its complete combustion. As indicated above the proper oxygen content can be attained by providing the constituents in direct proportion to their molecular weights and the number of molecules called for in their respective reaction equations.

The oxidizing agent that is used in the present invention is an organic oxidant, as distinguished for instance from hydrogen peroxide, and is preferably selected from the group of fully nitrated aliphatic compounds and comprises tetranitromethane  $\text{C}(\text{NO}_2)_4$  and hexanitroethane  $\text{C}(\text{NO}_2)_3\text{C}(\text{NO}_2)_3$ . A preferred combination to be selected comprises nitromethane as a fuel and tetranitromethane as an oxidant. These two ingredients are mixed in the following proportions by weight if a stoichiometric mixture is desired:

| Per cent                        |
|---------------------------------|
| Nitromethane ----- 55.5         |
| 45 Tetranitromethane ----- 44.5 |

Considerable variation in the above percentages is permissible without departing from the scope of the invention. For example if a mixture of nitromethane  $\text{CH}_3\text{NO}_2$  and tetranitromethane  $\text{C}(\text{NO}_2)_4$  falls within the percentages by weight given below it is considered that the resultant propellant lies within the bounds of the present invention:

| Per cent                      |
|-------------------------------|
| 55 Nitromethane ----- 25-75   |
| Tetranitromethane ----- 75-25 |

Thus it is contemplated that insofar as the proportions of fuel and oxidant are concerned a reasonable variation from the ideal calculated percentages is permissible and even desirable under certain conditions such as maintenance of desired combustion characteristics. The mixture of nitromethane and tetranitromethane emphasized above, while a preferred form of the invention, is intended to be illustrative of the variations in composition permissible herein. The other fuels and oxidants listed also may be used either in stoichiometric proportions or within the ranges hereafter set out.

Compositions in terms of percentage by weight are given below for other nitro and polynitro aliphatic fuels within the scope of the present invention, and for purposes of comparison the percentages of composition of the nitromethane

fuels are repeated. It should be pointed out that while it will generally be the case that the fuel component will consist of only one of the following ingredients it is contemplated to be within the scope of this invention to use in the propellant a fuel that contains one or more of these nitro and polynitro aliphatics. In such case the proposed proportions for stoichiometric mixtures may be arrived at in accord with the molecular weights and the reaction formula for the particular combination that is contemplated. Since these calculations lie within the ability of one skilled in this art they will not be given here.

When tetranitromethane is the oxidant that is used the following table indicates the percentages by weight of fuel that are to be used. In the first column the fuel is listed and in the second column the percentage by weight of a stoichiometric mixture of the fuel and tetranitromethane is desired. In the third column is listed the range of percentages by weight of fuel that will provide a satisfactory product when combined with tetranitromethane. In the case of both columns 2 and 3 the amount of tetranitromethane to be used may be obtained by subtracting from 100% the percentage of the fuel indicated. This table is as follows:

| Fuel                  | Fuel for Stoichiometric Mixture | Range of Percentages of Fuel |
|-----------------------|---------------------------------|------------------------------|
| nitromethane          | 55.5                            | 25-75                        |
| nitroethane           | 23.8                            | 15-50                        |
| 1-nitropropane        | 26.6                            | 10-40                        |
| 2-nitropropane        | 26.6                            | 10-40                        |
| 1,1-dinitropropane    | 45.8                            | 20-65                        |
| 2,2-dinitropropane    | 45.8                            | 20-65                        |
| 1,2-dinitropropane    | 45.8                            | 20-65                        |
| 1,3-dinitropropane    | 45.8                            | 20-65                        |
| 1,1-dinitroethane     | 65.5                            | 35-90                        |
| 1,1,1-trinitropropane | 68.7                            | 40-95                        |
| 1,2,3-trinitropropane | 68.7                            | 40-95                        |

If the oxidant to be used is hexanitroethane the following table governs in which again the first column is the fuel, the second column the percent by weight of fuel required for a stoichiometric mixture with hexanitroethane and the third column indicates the permissible range that may be used for a particular fuel. Again the amount of hexanitroethane to be added is obtained by subtracting from 100% the indicated percentage by weight of the fuel:

| Fuel                  | Fuel for Stoichiometric Mixture | Range of Percentages of Fuel |
|-----------------------|---------------------------------|------------------------------|
| nitromethane          | 52.2                            | 20-70                        |
| nitroethane           | 30.8                            | 10-45                        |
| 1-nitropropane        | 24.2                            | 10-40                        |
| 2-nitropropane        | 24.2                            | 10-40                        |
| 1,1-dinitropropane    | 42.5                            | 20-65                        |
| 2,2-dinitropropane    | 42.5                            | 20-65                        |
| 1,2-dinitropropane    | 42.5                            | 20-65                        |
| 1,3-dinitropropane    | 42.5                            | 20-65                        |
| 1,1-dinitroethane     | 62.3                            | 30-85                        |
| 1,1,1-trinitropropane | 65.6                            | 35-90                        |
| 1,2,3-trinitropropane | 65.6                            | 35-90                        |

Under certain conditions of use, mono nitro aliphatics are preferred. It is to be noted that mono nitro aliphatics are referred to herein simply as nitro aliphatics and that the prefix "mono" is not used—as for example mono nitromethane is referred to simply as nitromethane. On the other hand in the case of poly nitroaliphatics the prefixes, as "di," "tri" and "tetra" are used. These

mono nitroaliphatic compounds include the following:

Nitromethane,  $\text{CH}_3(\text{NO}_2)$   
 Nitroethane,  $\text{CH}_3\text{CH}_2\text{NO}_2$   
 1-nitropropane,  $\text{CH}_3\text{CH}_2\text{CH}_2\text{NO}_2$   
 2-nitropropane,  $(\text{CH}_3)_2\text{CH}\text{NO}_2$

This group of fuels may be used individually or they may be used in admixture with each other. An example of the latter is the fortuitous mixture of these compounds that results from the reaction of propane and nitric acid in the vapor or gas phase: see U. S. Patent 1,967,657, granted July 24, 1934, to H. B. Hass et al. Such a mixture may be used with an oxidant in stoichiometric proportions, in which case the fuel of this fortuitous mixture is mixed with tetranitromethane in approximately the following proportions by weight:

20 Per cent by weight  
 Tetranitromethane ----- 65  
 Fortuitous fuel mixture ----- 35

Again if the oxidant is hexanitroethane the corresponding mixture will be approximately as follows:

25 Per cent by weight  
 Hexanitroethane ----- 70  
 Fortuitous fuel mixture ----- 30

30 In each case, nitromethane, nitroethane, 1-nitropropane and 2-nitropropane are assumed to be present. Considerable latitude is permissible within the scope of the invention particularly when the fuel is such a fortuitous mixture as discussed above. Thus if the oxidant is tetranitromethane the propellants of this mixture that lie within the following percentages by weight are deemed to be within the present invention:

35 Per cent by weight  
 Fortuitous fuel mixture ----- 15-50  
 Tetranitromethane ----- 85-50

40 Again propellants using hexanitroethane as the oxidant and a fortuitous fuel mixture, if mixed in approximately the following ranges of percentage by weight, fall within the scope of this invention:

45 Per cent by weight  
 Hexanitroethane ----- 90-55  
 Fortuitous fuel mixture ----- 10-45

50 The combination of fuel and oxidant set out above may be used alone or in combination with still other ingredients and the addition of such other ingredients to a propellant mixture is contemplated as within the scope of this invention as defined in the claims. Such other ingredients may be in the form of a diluent or an inhibitor by which to control flame temperature, the rate of combustion and the like.

55 From the foregoing tables it will be seen that the invention broadly may comprise a nitro or polynitro aliphatic fuel and tetranitromethane in substantially the following range of percentages by weight:

60 Per cent  
 Tetranitromethane ----- 5-90  
 Nitro or polynitro aliphatic fuel ----- 95-10

65 and in the same manner the fuel and hexanitroethane may be used within the following range of percentages by weight:

70 Per cent  
 Hexanitroethane ----- 10-90  
 Nitro or polynitro aliphatic fuel ----- 90-10

75 The fuel and the oxidizing agent may be sup-

plied to the point of combustion as a mono-fuel that is already mixed and in liquid form. "Point of combustion" is a term not to be confined to the actual point of flame propagation but is construed to be the region to which the propellant is fed preparatory to the actual burning.

Although a preferred use of the present invention is in the form of a mono-fuel in which a single liquid entity is stored, transported and fed to the point of combustion, this is not necessary. In certain cases it is desirable to maintain the constituents separate from each other until they are brought together at the point of combustion. Such a procedure would be desirable if the combustion characteristics of the self-sufficient fuel were to be altered during use by altering the percentages in which the constituents are mixed at the point of combustion.

The propellant that is the subject of this invention may be used for various purposes and in various ways. Its use in a gas turbine or other prime mover has been emphasized here but it is not to be limited to such use. It may be used in any apparatus and environment where combustion of a fuel is employed as for instance a source of gas under pressure as by confined combustion of the propellant and retention of the products of combustion.

This application is a continuation in part of prior applications Serial No. 597,959, filed June 6, 1945, and Serial No. 640,386, filed January 10, 1946, both now abandoned.

I claim:

1. A self-sufficient liquid fuel comprising a compound selected from the group consisting of tetrannitromethane and hexanitroethane as an oxidizing agent and a liquid nitroparaffin as a fuel, the latter characterized by containing not more than one nitro group for each atom of carbon. 35

2. A self-sufficient liquid fuel comprising between five and ninety per cent by weight of tetrannitromethane as an oxidizing agent and the balance a liquid nitroparaffin as a fuel, the latter characterized by containing not more than one nitro group for each atom of carbon. 45

3. A self-sufficient liquid fuel comprising, in approximately stoichiometric proportions so as to give end products of carbon dioxide, water and nitrogen, tetrannitromethane as an oxidizing agent 50

and a liquid nitroparaffin as a fuel, the latter characterized by containing not more than one nitro group for each atom of carbon.

4. A prime mover propellant that comprises 25 to 75% by weight of nitromethane and 75 to 25% by weight of tetrannitromethane.

5. A propellant as in claim 4 consisting essentially of 25 to 75% of nitromethane and the balance tetrannitromethane.

10 6. A propellant as in claim 4 consisting essentially of 55.5% nitromethane and 44.5% tetrannitromethane.

15 7. A prime mover propellant comprising a plurality of homologous aliphatic nitro compounds, at least one of them consisting of a nitroparaffin of the nature of an oxidizing agent selected from the group consisting of tetrannitromethane and hexanitroethane and at least one of them consisting of a nitroparaffin of the nature of a fuel 20 having not more than one nitro group for each carbon atom appearing in the paraffin skeleton.

8. A propellant as in claim 7 including nitromethane as a fuel component.

25 9. A propellant as in claim 7 including a nitroethane fuel component.

10. A propellant as in claim 7 including a nitropropane fuel component.

15 11. A self-sufficient liquid fuel comprising a compound selected from the group consisting of tetrannitromethane and hexanitroethane as an oxidizing agent and, as fuel, a fortuitous mixture of mono nitroparaffins obtained by interacting propane and nitric acid in the vapor phase.

JOHN A. HANNUM.

#### REFERENCES CITED

The following references are of record in the file of this patent:

#### UNITED STATES PATENTS

| Number    | Name   | Date          |
|-----------|--------|---------------|
| 914,624   | Winand | Mar. 9, 1909  |
| 2,317,557 | Senkus | Apr. 27, 1943 |

#### FOREIGN PATENTS

| Number  | Country       | Date          |
|---------|---------------|---------------|
| 26,261  | Great Britain | 1907          |
| 248,548 | Germany       | June 25, 1912 |
| 24,839  | Great Britain | 1913          |